

## UNITED STATES PATENT OFFICE

2,203,080

## ELECTRICAL CONDUCTOR

Donald K. Crampton, Marion, Conn., assignor to  
 Chase Brass & Copper Co. Incorporated, Water-  
 bury, Conn., a corporation

No Drawing. Application August 11, 1938,  
 Serial No. 224,301

2 Claims. (Cl. 191—22)

This invention relates to improvement in electrical conductors formed of copper-base alloys, and more particularly to electrical trolley wires formed of such alloys.

5 One object of this invention is to produce electrical trolley wires formed of copper-base alloys, and having a combination of high electrical conductivity and high tensile strength.

Another object of this invention is to produce 10 electrical trolley wires formed of copper-base alloys and having a combination of high electrical conductivity, high tensile strength, and high resistance to wear.

Another object of this invention is to produce 15 electrical trolley wires formed of copper-base alloys and having a combination of high electrical conductivity, high tensile strength, and high resistance to wear and arcing.

Another object of this invention is to produce 20 electrical trolley wires formed of copper-base alloys and having a combination of high electrical conductivity, high tensile strength, high resistance to wear and arcing, and which can be produced at relatively-low cost.

25 The expression, "combination of high electrical conductivity and high tensile strength," in this application, does not necessarily mean that each is particularly high, considered alone, but that the combination of the properties is attractive or high from a practical standpoint. Thus, for example, the conductivity is high for a given tensile strength, or vice versa.

I have found that trolley wires can be given a combination of high electrical conductivity, high tensile strength, and high resistance to wear and to arcing and can be formed at a relatively-low cost when containing by weight, zinc from about 8% to about 12%, and the balance substantially of copper, it being understood that the 30 alloy may contain minor amounts of impurities of such metals, for example, as lead, iron, aluminum, tin, silicon, and so forth, provided the total of such impurities is not sufficient to lower the conductivity below the permissible desired limit. One preferred electrical trolley wire, in accordance with the present invention, has the zinc content about 10%.

In casting ingots from alloys in accordance with the present invention, no harmful segregation occurs. Also, it is unnecessary to use any deoxidizing agent in casting the ingots, thus avoiding undue reduction of the electrical conductivity caused by deoxidizing agents. 5

When the ingots are reduced to the form of drawn trolley wires, in accordance with the well-known and usual processes, these trolley wires are found to have exceptional resistance to wear 10 from the rubbing action of trolley wheels and shoes and the like, and also to have exceptional resistance to wear or destruction due to the formation of electrical arcs between the trolley wire and the trolley wheel or shoe. Another important fact is that the cost of the zinc and copper for making the alloy is relatively low and the cost of the fabricating processes is also relatively low, due to the ease of working this alloy. 15

The invention may be carried out in other 20 specific ways than those therein set forth without departing from the spirit and essential characteristics of the invention, and the present embodiments are, therefore, to be considered in all respects as illustrative and not restrictive, and all changes coming within the meaning and equivalency range of the appended claims are intended to be embraced therein. 25

I claim:

1. An electrical trolley wire characterized by 30 a combination of high conductivity, high tensile strength, ease of working, low cost, high resistance to wear and high resistance to arcing, and formed of a copper-base alloy consisting of zinc from about 8% to about 12% and the balance of 35 copper except for impurities.

2. An electrical trolley wire characterized by 40 a combination of high conductivity, high tensile strength, ease of working, low cost, high resistance to wear and high resistance to arcing, and formed of a copper-base alloy consisting of zinc about 10% and the balance of copper except for impurities.

DONALD K. CRAMPTON.

45